

# United States Patent Office

3,234,031

Patented Feb. 8, 1966

1

3,234,031

## REDUCTION NICKEL PLATING WITH BORON REDUCING AGENTS AND ORGANIC DIVALENT SULFUR STABILIZERS

Eberhard Zirngiebl, Cologne-Flittard, and Heinz Günther Klein, Cologne-Deutz, Germany, assignors to Farbenfabriken Bayer Aktiengesellschaft, Leverkusen, Germany, a corporation of Germany

No Drawing. Filed Jan. 22, 1962, Ser. No. 167,959  
Claims priority, application Germany, Feb. 4, 1961,

F 33,143

8 Claims. (Cl. 106—1)

The present invention is directed to an improved process of chemical metal plating of metal and plastic articles employing an aqueous bath containing salts of the metals to be deposited and boron compounds as reducing agents.

Chemical plating baths for the production of metal coatings on metal or plastic surfaces are known. As coating metals there are chiefly used nickel and/or cobalt, but iron or zinc can also be deposited together with nickel and/or cobalt. Known reducing agents are, besides alkali metal hypophosphites chiefly boron compounds with 1—4 hydrogen atoms directly linked with boron, for example, alkali metal borohydrides or alkylamine boranes. In order to increase the plating rate and the reduction yield, salts or other compounds of metals of Groups IIb, IIIb, IVb, Vb, and/or VIb of the Periodic System of Elements may be added to these baths.

However, it has been found that these baths tend to separate out metal flakes or to decompose with the formation of a black precipitate as soon as the concentration of the baths in plating metal has dropped by about 10 to 25% in the course of plating. In some cases these baths can be further used after filtration, but in most cases the plating stops after a short time and the baths must be discarded or worked up. For example, a bath of the composition: 30 g./liter of nickel chloride, 40 g./liter of sodium hydroxide, 50 g./liter of ethylenediamine, 0.6 g./liter of sodium borohydride, decomposes after 19.3% of the nickel employed have been used up from the bath by plating. Even after filtration of this bath, no further plating takes place.

It is an object of this invention to provide an improved process for chemical metal plating of metal and plastic surfaces and an improved bath for use in the chemical metal plating of plastic and metal articles containing a salt of the metal to deposit and a boron compound with 1—4 hydrogen atoms directly linked with the boron.

It is also an object of this invention to provide an improved bath containing metal salts as additive, said metals being from the Groups IIb, IIIb, IVb, Vb, and VIb of the Periodic System of Elements.

It has been discovered that the adding of a small effective amount of an organic bivalent sulfur compound, which is soluble in the bath liquid and wherein each of the two valencies of the sulfur atom are directly linked with a carbon atom produces a particularly good stabilizing effect.

Acidic baths moreover may contain buffer substances known as such, alkaline baths may contain complex formers known as such and, if desired, buffer substances. In order to increase the reduction yield and/or plating rate, these baths may furthermore contain additives of chemically linked metals of Groups IIb, IIIb, IVb, Vb, and VIb of the Periodic System of Elements.

The presence of organic sulfur compounds with formally bivalent sulfur in a plating bath containing as reducing agent borohydride compounds with 1 to 4 hydrogen atoms directly linked with boron and in addition thereto metal salts as additives, said metals being from the Groups IIb, IIIb, IVb, Vb, and VIb of the Periodic System of

2

Elements has been found to exert such a stabilizing effect on the bath that the process of chemical metal plating may be executed continuously. For example, a nickel bath with an optimum concentration in nickel salt

(NiCl<sub>2</sub>·6H<sub>2</sub>O)

and alkali metal borohydride (NaBH<sub>4</sub>) decomposes as soon as about 25% of the initial nickel content have been consumed by the plating process using a ratio of surface (in sq. cm.) bath volume (in cc.), S/V=0.4. When 1.6 g./liter of thio-diglycollic acid are added to a bath of the same initial concentration using the same ratio S/V, no decomposition takes place even after a deposition of over 50% of the metal by plating.

15 The reduction yields, referred to the boron compound as well as to the metal salt, are likewise substantially improved by the addition of organic sulfur compounds soluble in the bath liquid. For example, with a nickel bath having an initial concentration of 30 g./liter of nickel chloride, 40 g./liter of sodium hydroxide, 50 g./liter of ethylenediamine, 0.59 g./liter of sodium borohydride, the following values are obtained for the reduction yield as a function of the quantity of nickel deposited by plating:

| Deposited nickel,<br>percent: | Reduction yield,<br>percent |
|-------------------------------|-----------------------------|
| >0—10.76                      | 21.82                       |
| 10.76—18.89                   | 16.55                       |
| 18.89—25.20                   | 12.84                       |

### 30 Decomposition of the bath.

With a bath of the same composition containing, in addition, 1.6 g./liter of thioglycollic acid, the following values are obtained:

| Deposited nickel,<br>percent: | Reduction yield,<br>percent |
|-------------------------------|-----------------------------|
| >0—15.35                      | 31.15                       |
| 15.35—30.55                   | 30.82                       |
| 30.55—43.60                   | 26.55                       |
| 43.60—52.95                   | 18.86                       |
| 52.95—64.30                   | 23.12                       |
| 64.30—75.65                   | 23.05                       |

### 35 No decomposition of the bath.

These values are established after 0.59 g. of sodium borohydride have been used up for plating in each test.

45 The addition of organic sulfur compounds with formally bivalent sulfur to chemical plating baths leads not only to a considerable stabilization of the baths, but, in the case where mixed cobalt-nickel baths are used, also to a preferred deposition of nickel. For example, a solution of 45 g. Ni(NH<sub>3</sub>)<sub>6</sub>Cl<sub>2</sub>, 5 g. CoCl<sub>2</sub>·6H<sub>2</sub>O, 5 g. NH<sub>4</sub>Cl and 1 g. NaBH<sub>4</sub> in 1 liter of 2 N ammonia solution yields at 50° C. on metal or plastic surfaces a Co-Ni-B coating containing 9.8% of nickel. From a bath of the same composition containing, in addition, 1.0 g./liter of 3,4-diphenylthiophene-dicarboxylic acid, there is obtained at 50° C. on metal or plastic surfaces a Co-Ni-B coating in which 31.7% of nickel can be detected.

50 As examples of organic sulfur compounds with formally bivalent sulfur, wherein the sulfur atom is directly linked with carbon atoms, used according to the invention there may be mentioned.

55 (1) Sulfur-containing aliphatic carboxylic acids, alcohols and their derivatives:



3



## (2) Sulfur-containing aromatic/aliphatic carboxylic acids:



## (3) Sulfur-containing acetylene compounds:



## (4) Aromatic sulfides:



## (5) Thiophenes, thionaphthalenes:



## (6) Thiazoles:





The organic sulfur compounds can be added to the plating baths individually or as mixtures. It is frequently of advantage to add one or more metal salts of Groups of IIb, IIIb, IVb, Vb and/or VIb of the Periodic System of Elements to the plating bath, in addition to the organic sulfur compounds. With these new baths metal and plastic surfaces can be plated more satisfactorily and economically than has hitherto been possible. The content of the baths in salts of the plating metals such as chlorides, sulphates, acetates etc. of, for example, nickel, cobalt, nitrates and formates corresponds to the values already known from borohydride- or borazane-containing baths. As reducing agents for the chemical depositing of metal there may be used for example:

(1) Alkali metal borohydrides; e.g. sodium borohydrides;

(2) Water-soluble BH-compounds; e.g. trimethylamine borane, dimethylamine borane, dimethylaminoborane;

(3) BH-compounds which have been rendered water-soluble by the addition of solubilizers; e.g. diethylamine borane, isopropylamine borane etc.

Suitable solubilizers, for example, are methanol, ethanol, dioxan etc. As buffer substances for these new plating baths there may be used, for example, sodium acetate, sodium citrate, sodium tartrate etc. Suitable complex formers, for example, are ammonia and amines such as ethylene-diamine, ethanol-amine, tetramethylene diamine, diethylene triamine, triethylene tetramine, ethylenediamino tetraacetic acid, nitrilotriacetic acid.

The following Table 1 summarizes the basic concentration range of the bath components in accordance with this invention.

Table 1

| Compounds                                                    | Concentration range in the bath liquid |         |
|--------------------------------------------------------------|----------------------------------------|---------|
|                                                              | Mols/l.                                | G/l.    |
| Plating metal salts                                          | 0.02-0.5                               | 0.1-5   |
| Alkali metal borohydride                                     |                                        |         |
| Water-soluble boron compounds e.g. sodium tetraborate        | 0.1-10                                 |         |
| Other boron compounds e.g. alkyl amino boranes and borazoles | 0.1-10                                 |         |
| Metal salts as additives                                     | 0.2-5                                  | 0.001-1 |
| Complex formers                                              |                                        | 5-200   |
| Buffer substances                                            |                                        | 0.001-5 |
| Organic sulfur compounds                                     |                                        |         |

Although the organic sulfur compounds, when incorporated in the plating bath, may be used in concentrations as high as 5 g./l., there is no improvement to be gained from the higher concentrations, and they are preferably used in the range of concentrations from about 0.01 to 1 g./l. Metals such as nickel copper alloys, aluminum, iron as well as plastic material such as films, sheetings, plates, fabrics and moulding articles from acetyl cellulose, cellulose-acetobutyrate, polyvinyl-chloride, polyamides, polyurethanes, polystyrene, polycarbonates, polyacrylates, polyethylene and polypropylene. The surface of these plastic articles may be activated by treating said surface with acids, alkali and metal salts, prior to plating.

The following examples illustrate the applicability of using the organic sulfur compound in chemical plating baths according to the invention.

## EXAMPLE 1

In each of 5 chemical plating baths (a), (b), (c), (d), and (e) each of which contains 1 liter of bath liquor

consisting of 30 g./liter of nickel chloride, 40 g./liter of sodium hydroxide and 50 g./liter of ethylene-diamine, there are suspended 2 weighed copper and 2 brass plates with a surface of 1 sq. dm./plate. To the baths (b), (c), (d), and (e) are added (b)=0.2 g., (c)=0.4 g., (d)=0.8 g. and (e)=1.6 g. of thioglycollic acid. The bath (a) contains no addition of thioglycollic acid. The baths are heated to 90° C. and to each bath is added 0.59 g. of 100% sodium borohydride previously dissolved in about 50 cc. of the bath liquor. The plating of the metal plates sets in immediately after the addition of the reducing agent. After a plating time of 40 minutes, sodium borohydride can no longer be detected in any bath by iodometric analysis. Subsequently the plates are removed from the plating baths, rinsed, dried and the increase in weight is established.

In all of the plating baths there are again suspended two weighed plates each of copper and brass and 0.59 g. of sodium borohydride are added at 90° C. to all of the baths. This process is repeated six times. The following weights of deposited nickel are obtained from which the percentage of nickel deposited from the bath and the reduction yields for each addition of reducing agent can be calculated.

## BATH (a) (WITHOUT ADDITION OF THIODIGLYCOLIC ACID)

| Deposited Ni/4 plates, g.  | Deposited Ni, percent | Reduction yield, percent |
|----------------------------|-----------------------|--------------------------|
| 0.7966                     | 10.76                 | 21.82                    |
| 0.6049                     | 18.89                 | 16.55                    |
| 0.4637<br>( <sup>1</sup> ) | 25.20                 | 12.84                    |

## BATH (b) (0.2 G. THIODIGLYCOLIC ACID)

|                            |       |       |
|----------------------------|-------|-------|
| 0.9340                     | 12.6  | 25.6  |
| 0.7645                     | 22.9  | 20.95 |
| 0.6125                     | 31.2  | 16.78 |
| 0.3696                     | 36.2  | 10.12 |
| 0.5084                     | 43.0  | 16.0  |
| 0.4464<br>( <sup>2</sup> ) | 49.05 | 12.24 |

## BATH (c) (0.4 G. THIODIGLYCOLIC ACID)

|                            |       |       |
|----------------------------|-------|-------|
| 0.9365                     | 12.65 | 25.69 |
| 0.6542                     | 21.48 | 17.93 |
| 0.7160                     | 31.9  | 19.63 |
| 0.4412                     | 37.1  | 12.1  |
| 0.5802                     | 44.9  | 15.9  |
| 0.4880<br>( <sup>2</sup> ) | 51.5  | 13.37 |

## BATH (d) (0.8 G. THIODIGLYCOLIC ACID)

|                            |       |       |
|----------------------------|-------|-------|
| 1.1471                     | 15.43 | 31.4  |
| 0.9086                     | 27.73 | 24.9  |
| 0.8141                     | 38.7  | 22.3  |
| 0.5608                     | 46.3  | 15.38 |
| 0.6344                     | 54.8  | 17.37 |
| 0.6010<br>( <sup>2</sup> ) | 62.9  | 16.47 |

## BATH (e) (1.6 G. THIODIGLYCOLIC ACID)

|        |       |       |
|--------|-------|-------|
| 1.1375 | 15.35 | 31.15 |
| 1.1255 | 30.55 | 30.82 |
| 0.9690 | 43.60 | 26.55 |
| 0.6884 | 52.95 | 18.86 |
| 0.8440 | 64.30 | 23.12 |
| 0.8404 | 75.65 | 23.05 |

<sup>1</sup> Bath is decomposed. <sup>2</sup> No decomposition.

## EXAMPLE 2

To three chemical plating baths (a), (b) and (c) of the composition described in Example 1 and a bath volume of 1 liter there is added to bath (b)=0.08 g., to bath (c)=0.16 g. of acetylene-dithiosalicylic acid. Bath (a) contains no stabilizer. The S/V ratio is 0.4. The working method is the same as in Example 1. The fol-

lowing values are obtained for the reduction yield as a function of the quantity of nickel deposited by plating.

BATH (a) (WITHOUT ADDITION OF ACETYLENE-DITHIOSALICYLIC ACID)

| Deposited Ni, percent: | Reduction yield, percent |
|------------------------|--------------------------|
| >0-10.02               | 20.32                    |
| 10.02-18.37            | 16.95                    |
| 18.37-19.94            | 3.20                     |
| Decomposition.         | 10                       |

BATH (b) (0.08 G. ACETYLENE-DITHIOSALICYLIC ACID)

| Deposited Ni, percent: | Reduction yield, percent |
|------------------------|--------------------------|
| >0-13.92               | 28.25                    |
| 13.92-27.85            | 28.18                    |
| 27.85-40.65            | 26.09                    |
| 40.65-50.5             | 19.97                    |
| 50.5-59.2              | 17.74                    |
| No decomposition.      |                          |

BATH (c) (0.16 G. ACETYLENE-DITHIOSALICYLIC ACID)

| Deposited Ni, percent: | Reduction yield, percent |
|------------------------|--------------------------|
| >0-8.74                | 17.75                    |
| 8.74-27.6              | 37.18                    |
| 27.6-42.9              | 32.18                    |
| 42.9-56.0              | 26.75                    |
| 56.0-72.2              | 32.6                     |
| No decomposition.      |                          |

EXAMPLE 3

In 1 liter of a chemical plating bath of a composition of 30 g./liter of nickel chloride, 40 g./liter of sodium hydroxide, 50 g./liter of ethylenediamine, 20 mg./liter of lead chloride, 160 mg./liter of 3-hydroxy-thionaphthene-carboxylic acid-(2), there are suspended 4 iron plates with a surface of 1 sq. dm./plate. The plates are previously weighed. The bath is heated to 90° C. and treated with about 50 cc. of bath liquor containing 0.6175 g. 100% NaBH<sub>4</sub> in solution. At intervals of 30 minutes one plate is withdrawn from the bath and a new weighed plate as well as 0.6175 g. NaBH<sub>4</sub> are added to the bath. The proportion S/V=0.4 is thus not changed. The experiment is continued for a period of 2 hours. The bath volume is maintained constant by replacing the evaporated water. The total NaBH<sub>4</sub> consumption amounts to 4×0.6175 g. 50 = 2.4700 g. This corresponds to a theoretically possible nickel deposit of 15.284 g. There are deposited:

|                             | G./sq. dm. |
|-----------------------------|------------|
| After a stay of 30 minutes  | 0.4108     |
| After a stay of 60 minutes  | 0.6898     |
| After a stay of 90 minutes  | 0.9602     |
| After a stay of 120 minutes | 1.1719     |
| After a stay of 90 minutes  | 0.8326     |
| After a stay of 60 minutes  | 0.5601     |
| After a stay of 30 minutes  | 0.3152     |

The total Ni deposit (4.9406 g.) corresponds to a reduction yield of 32.35%, calculated on the NaBH<sub>4</sub> consumption. 66.7% of the nickel present in the plating bath are deposited without decomposition of the bath.

EXAMPLE 4

In 1 liter of a chemical plating bath of a composition of 30 g./liter of nickel chloride, 40 g./liter of sodium hydroxide, 60 g./liter of ethylenediamine, 0.2 g./liter of thioglycollic acid, 0.1 g./liter of S-(2-carboxyphenyl)-thioglycollic acid, there are suspended 4 weighed iron plates with a surface of 1 sq. dm./plate. The addition of sodium borohydride is 0.5795 g. each time. The working

75

method corresponds to that of Example 1. The following values are obtained:

| Deposited Ni/4 plates, g. | Deposited Ni, percent | Reduction yield, percent |
|---------------------------|-----------------------|--------------------------|
| 0.9813                    | >0-13.24              | 27.5                     |
| 0.8003                    | 13.24-24.03           | 22.35                    |
| 0.6827                    | 24.03-33.5            | 19.15                    |
| 0.6285                    | 33.5-41.75            | 17.56                    |
| 0.5745                    | 41.75-49.45           | 16.05                    |
| 0.5256                    | 49.45-56.59           | 14.68                    |

EXAMPLE 5

Acetyl-cellulose foils are successively treated in the following baths:

- (a) 100 g. of sodium hydroxide + 0.3 g. of wetting agent + 900 g. of water  
Time of stay: 5 minutes, temperature 50-60° C.
20. (b) 100 g. of stannous chloride + 200 cc. of conc. hydrochloric acid + 0.2 g. of wetting agent + 850 cc. of water  
Time of stay: 5 minutes, temperature 50-60° C.
- (c) 0.5 g./liter of palladium chloride + 10 cc./liter of conc. hydrochloric acid  
Time of stay: 5 minutes, temperature 20-30° C.

Four foils with a thickness of 100 $\mu$  and a surface of 1 sq. dm./foil pre-treated in this way are suspended in a bath heated to 70° C. and having a composition of 30 g. of nickel chloride, 5 g. of ammonium chloride, 10 g. of sodium citrate, 20 g. of sodium acetate, 150 mg. of S-(2-carboxyphenyl)-thioglycollic acid. The pH value is 5.0. After the addition of 50 ml. of a solution of 3.55 g. of diethylamine borane in methanol, a brilliant Ni-B coating is obtained on all foils. Every 45 minutes the foils from the bath are exchanged for 4 new foils, another 3.55 g. of diethylamine borane in 50 ml. of methanol being added every time. The consumption of amine borane per throughput is determined by iodometric analysis. This process is repeated five times. The reduction yields are determined by means of the deposited amount of Ni and the consumption of amine borane per charge. The values for a bath of the same composition conducted in the same way without an addition of organic sulfur compound are given for comparison. The following values are obtained:

(1) BATH WITHOUT ADDITION

| Deposited nickel, percent: | Reduction yield, percent |
|----------------------------|--------------------------|
| >0-18.24                   | 20.0                     |
| 18.24-32.7                 | 14.15                    |
| 32.7-48.4                  | 16.33                    |
| 48.4-61.78                 | 13.82                    |
| 61.78-74.9                 | 14.38                    |

After the first and second charge the bath liquor has to be filtered because of metal flakes separating out.

(2) BATH WITH ADDITION OF 150 MG./LITER OF S-(2-CARBOXYPHENYL)-THIOLYCOLIC ACID

| Deposited nickel, percent: | Reduction yield, percent |
|----------------------------|--------------------------|
| >0-13.45                   | 28.39                    |
| 13.45-37.31                | 16.76                    |
| 37.31-54.2                 | 17.05                    |
| 54.2-68.3                  | 14.23                    |
| 68.3-79.1                  | 12.15                    |

EXAMPLE 6

In each of four chemical plating baths (a), (b), (c) and (d) consisting of 15 g. of cobalt chloride, 15 g. of nickel chloride, 5 g. of ammonium chloride, 20 g. of sodium acetate and 950 cc. of water there are suspended two weighed plates each of copper and brass with a surface of 1 sq. dm./plate. To the baths (b), (c) and (d) there are added (b)=50 mg., (c)=100 mg. and (d)=150 mg. of thioglycollic acid. The bath (a) contains no

addition of thioldiglycollic acid. The baths are heated to 70° C. and 50 ml. of a solution of 3.55 g. of diethylamine borane in methanol are added to each bath. The pH value of the plating baths is 5.0. Every 45 minutes the plates are exchanged for new metal plates, another 3.55 g. of diethylamine borane in 50 cc. of methanol being added each time. The consumption of diethyl amine borane is determined iodometrically. This process is repeated four times. It can be seen already from the coloration of the baths, that cobalt is preferably deposited in the baths (a) and (b), whereas nickel is preferably deposited in the baths (c) and (d). The metal coating deposited on the metal plates is removed with nitric acid and analysed as to its cobalt and nickel content. The reduction yields are established by means of the consumption of amine borane per charge and of the metal deposition on the copper and brass plates.

BATH (A) (WITHOUT ADDITION OF THIODIGLYCOLIC ACID)

[The plating bath must be filtered after the first and second charge from the separated metal flakes]

| Deposited Ni-Co, percent | Reduction yield, percent | Co, percent | Ni, percent | B, percent |
|--------------------------|--------------------------|-------------|-------------|------------|
| >0-14.78                 | 15.46                    | 75.0        | 18.6        | 6.4        |
| 14.78-33.25              | 19.1                     | 66.4        | 28.1        | 5.5        |
| 33.25-49.4               | 16.55                    | -----       | -----       | -----      |
| 49.4-62.2                | 14.25                    | -----       | -----       | -----      |

BATH (B) (ADDITION OF 50 MG./LITER OF THIODIGLYCOLIC ACID)

[The bath is filtered after the second charge (few metal flakes)]

| Deposited Ni-Co, percent | Reduction yield, percent | Co, percent | Ni, percent | B, percent |
|--------------------------|--------------------------|-------------|-------------|------------|
| >0-19.8                  | 28.8                     | 51.7        | 43.9        | 4.4        |
| 19.8-41.2                | 17.9                     | -----       | -----       | -----      |
| 41.2-57.1                | 15.9                     | 52.3        | 42.8        | 4.9        |
| 57.1-70.3                | 13.5                     | -----       | -----       | -----      |

BATH (C) (ADDITION OF 100 MG./LITER OF THIODIGLYCOLIC ACID)

[Bath needs not to be filtered]

| Deposited Ni-Co, percent | Reduction yield, percent | Co, percent | Ni, percent | B, percent |
|--------------------------|--------------------------|-------------|-------------|------------|
| >0-19.6                  | 30.0                     | 41.7        | 55.6        | 2.7        |
| 19.6-45.4                | 21.45                    | -----       | -----       | -----      |
| 45.4-57.7                | 17.9                     | 46.7        | 51.3        | 2.0        |
| 57.7-71.8                | 16.2                     | -----       | -----       | -----      |

BATH (D) (ADDITION OF 150 MG./LITER OF THIODIGLYCOLIC ACID)

[Bath needs not to be filtered]

| Deposited Ni-Co, percent | Reduction yield, percent | Co, percent | Ni, percent | B, percent |
|--------------------------|--------------------------|-------------|-------------|------------|
| 0-16.65                  | 29.4                     | 30.8        | 68.0        | 1.2        |
| 16.65-40.75              | 22.4                     | 46.2        | 52.4        | 1.4        |
| 40.75-52.4               | 16.3                     | 41.7        | 55.6        | 2.7        |
| 52.4-64.5                | 13.5                     | -----       | -----       | -----      |

EXAMPLE 7

To four chemical plating baths (a), (b), (c) and (d), each of which contains 45 g./l. of nickel chloride, 2.5 g./l. of sodium tetraborate, 160 ml./l. of aqueous 25 percent solution of ammonia and 1 g./l. of sodium borohydride in a bath volume of 1 liter there is added to the bath (a) 1.0 g., to bath (b) 0.5 g. and to bath (c) 0.2 g. of 3,4-diphenyl-thiophene-2,5-dicarboxylic acid. The bath temperature is 45° C. In each of the baths there are suspended the weighted plates consisting of brass, copper and iron with a surface of 1 sq. dm./plate. The proportion S/V of the bath is 0.3. After a plating time of 45 minutes, the plates have been removed from the plating baths and the increase in weight (deposited nickel) is established.

| Bath      | Sulfur compound, g./l. | Deposited nickel, g. | Stability                       |
|-----------|------------------------|----------------------|---------------------------------|
| (a) ----- | 1.0                    | 1.2828               | No decomposition.               |
| (b) ----- | 0.5                    | 1.1738               | Do.                             |
| (c) ----- | 0.2                    | 1.0542               | Do.                             |
| (d) ----- | -----                  | 0.2735               | Decomposition after 15 minutes. |

EXAMPLE 8

To four chemical plating baths (a), (b), (c), and (d) of the composition described in Example 7, there are added the following amounts of the sulfur compound represented by the formula:



bath (a) 0.1 g., bath (b) 0.06 g., bath (c) 0.02 g. and bath (d) 0 g.

40 The procedure is according to Example 7.

| Bath      | Sulfur compound, g./l. | Deposited nickel, g. | Stability                       |
|-----------|------------------------|----------------------|---------------------------------|
| (a) ----- | 0.1                    | 1.274                | No decomposition.               |
| (b) ----- | 0.06                   | 1.382                | Do.                             |
| (c) ----- | 0.02                   | 1.218                | Do.                             |
| (d) ----- | -----                  | 0.249                | Decomposition after 12 minutes. |

EXAMPLE 9

55 In each of three chemical plating baths (a), (b), (c), of the composition of 31 g./l. of nickel chloride, 45 g./l. of sodium hydroxide, 65 g./l. of ethylene-diamine and 0.6 g./l. of sodium borohydride are suspended four weighted copper plates with a surface of 1 sq. dm./plate. To the baths (a) and (c) are added 0.01 g. and 0.016 g. of 4,4'-60 dinitro-diphenylsulfide-6,6'-disulfonic acid, bath (a) contains no organic sulfur compound. The procedure is according to Example 1. Bath (a) is decomposed, when 14.5 percent of the nickel has been deposited. The baths (b) and (c) do not show any decomposition, when 50 percent of the nickel has been deposited.

65 Example 10

70 The chemical plating baths according to Example 7 show a decomposition after 20 minutes of working time. A measure for the stabilization effect of the organic sulfur compounds mentioned in the Table 2 is the stability of these chemical plating baths containing said organic sulfur compounds in a bath composition according to Example 7.

| Structure                                  | Sulfur compound concentration, g./l. | Stability/working time in hours |
|--------------------------------------------|--------------------------------------|---------------------------------|
| <chem>S-C(=O)CH2</chem>                    | 0.1                                  | More than 1.                    |
| <chem>S-C(=O)CH2-C(=O)O</chem>             | 0.5                                  | Do.                             |
| <chem>S-(CH2)3CONH(CH2)3-OH</chem>         | 0.5                                  | 10 Do. 15                       |
| <chem>S-CH2-CH2-COON</chem>                | 0.5                                  | Do. 20                          |
| <chem>S-CH2-CH2-COOH</chem>                | 0.5                                  | Do. 25                          |
| <chem>CH(OH)-CCl3</chem>                   | 0.5                                  | Do. 30                          |
| <chem>S-CH(OH)-CCl2</chem>                 | 0.1                                  | Do. 35                          |
| <chem>Cl-C6H4-Cl-S-CH2-COOH</chem>         | 1.0                                  | Do. 40                          |
| <chem>CH(OH)-CH3</chem>                    | 0.1                                  | Do. 45                          |
| <chem>S-CH(OH)-CH3</chem>                  | 0.1                                  | Do. 50                          |
| <chem>Cl-C10H10-S-CH2-COOH</chem>          | 0.1                                  | Do.                             |
| <chem>SO3H-C6H4-N=C6H4-S-C6H4-NH2</chem>   | 0.1                                  | Do.                             |
| <chem>CH3-C6H4-N=C6H4-SO3H-C6H4-NH2</chem> | 0.1                                  | Do.                             |
| <chem>CH3-C6H4-N=C6H4-SO3H-C6H4-NH2</chem> | 0.05                                 | Do.                             |

Example 11

In a chemical plating bath, which has a temperature of 90° C. and contains per liter bath liquid 30 g. of nickel chloride ( $\text{NiCl}_2 \cdot 6\text{H}_2\text{O}$ ), 62 g. of ethylene diamine, 42 g. of sodium hydrazide, 1.0 g. of thio-diglycolic acid, 0.01 g. of lead chloride and 0.6 g. of sodium borohydride are suspended four metal plates. The proportion surface/volume of bath is 0.4.

Each half an hour one plate is withdrawn and a new plate is suspended, so that the time of stay of the first plate in the plating bath is amounted to half an hour, the second plate one hour, the third plate two hours and each of the following plates two hours.

Continuously there are added 100 cm.<sup>3</sup> per hour of a sodium borohydride solution consisting of 12 g. sodium borohydride and 1 liter of a 2 n aqueous solution of sodium hydroxide and 100 cm.<sup>3</sup> per hour of a metal salt solution consisting of 118 g./l. of nickel chloride ( $\text{NiCl}_2 \cdot 6\text{H}_2\text{O}$ ), 60 g./l. of ethylene-diamine, 1 g./l. of thioglycolic acid and 0.1 g./l. of lead chloride. Continuously 100 cm.<sup>3</sup> of the bath liquid has been withdrawn per hour.

After 10 hours' working time one liter of sodium borohydride solution and one liter of the solution of metal

salts are added to the plating bath and accordingly one liter is withdrawn. 24.1836 g. of nickel has been deposited and the consumption of sodium borohydride amounts to 12.0 g., corresponding to a reduction yield of 32 percent, calculated on nickel without decomposition of the bath liquid. The resulting plates show a silver luster.

What we claim is:

1. An aqueous metal and plastic plating bath for plating by chemical reduction consisting essentially of an aqueous solution of

(1) a plating metal selected from the group consisting of nickel, cobalt, and mixtures thereof in an amount of between 0.02 and 0.5 mol per liter;

(2) a boron compound selected from the group consisting of alkali metal borohydrides, trimethyl amine borane, dimethyl amine borine, dimethyl amine borane, diethyl amine borane, and isopropyl amine borane in an amount of between 0.1 and 10 g. per liter as reducing agent for said solution;

(3) a complex forming agent selected from the group consisting of ammonia, ethylene diamine, ethanol amine, tetramethylene diamine, diethylene triamine, triethylene tetra-amine, ethylene diamino-tetra-acetic acid, and nitrilo-triaceic acid in an amount of between 0.2 and 5 mols per liter; and

(4) at least one organic divalent sulfur compound selected from the group consisting of thio-diglycolic acid,  $\beta$ -thio-dipropionic acid, 1,1'-thio-bis-(2,2,2-trichloro-ethanol), (methylene-dithio)-diacetic acid, 1-ethyl-thioethanol, 2,2'-thio-diethanol,  $\alpha$ -amino- $\gamma$ -(methyl-thio)-butyric acid, bis-(N- $\gamma$ -oxypropyl)-thio-dipropylene glycol-dicarboxylic acid amide, S-(2-carboxyphenyl)-thio-glycolic acid, S(8-chloro-1-naphthyl)-thioglycolic acid, (p-chlorophenyl-thio)-acetic acid, (2-methyl 3-chlophenyl-thio)-acetic acid, (pentachlorophenyl - thio) - acetic acid, (2-nitro-4-acetamidophenyl-thio)-acetic acid, 2-( $\alpha$ -hydroxyethyl-thio)-4-ethylbenzoic acid, 3-carboxymethyl-thio-2-anthraquinone carboxylic acid (di-Na-salt), acetylene-dithio-salicylic acid, 4,4'-dinitro-diphenylsulfide-6,6'-disulfonic acid, 2,2'-thio-di(5-amino-benzene sulfonic acid), 2-thiophene carboxylic acid, 3,4-diphenyl-thiophene-2,5-dicarboxylic acid, 3-hydroxy-thionaphthene-2-carboxylic acid, 2-hydroxy-thionaphthene, 2 - hydroxy - 3 - dibenzo - thiophene-carboxylic acid, 2,3-thionaphthenedion, 2-(p-aminophenyl)-5-sulfo-6-benzothiazole carboxylic acid, 2-amino - 5 - (6'-methyl-2'-benzothio-azolyl)-1,3-benzene disulfonic acid, 2-(m-aminophenyl)-7-hydroxy-naphtho-(2,3-d)thioazole-5-sulfonic acid in an amount of between 0.001 and 5 g. per liter.

2. An aqueous metal and plastic plating bath according to claim 1 additionally containing a member selected from the group consisting of methanol, ethanol, and dioxane as solubilizer.

3. An aqueous metal and plastic plating bath according to claim 1 additionally containing a member selected from the group consisting of sodium acetate, sodium nitrate, and sodium tartrate in an amount of between 5 and 200 g. per liter, as buffering agent.

4. An aqueous metal and plastic plating bath according to claim 1 additionally containing in solution a lead salt in an amount of between 0.001 and 1 g. per liter.

5. Process for applying a metal coating to the surfaces of metal and plastic articles by chemical reduction consisting essentially of contacting the surfaces of such a metal and plastic article with a plating bath consisting essentially of an aqueous solution of

(1) a plating metal selected from the group consisting of nickel, cobalt, and mixtures thereof in an amount of between 0.02 and 0.5 mol per liter;

(2) a boron compound selected from the group consisting of alkali metal borohydrides, trimethyl amine

13

borane, dimethyl amine borine, dimethyl amine borane, diethyl amine borane and isopropyl amine borane in an amount of between 0.1 and 10 g. liter as reducing agent for said solution,

(3) a complex forming agent selected from the group consisting of ammonia, ethylene diamine, ethanol amine, tetra-methylene diamine, diethylene triamine, triethylene tetra-amine, ethylene diamino-tetra-acetic acid, and nitrilo-triacetic acid in an amount of between 0.2 and 5 mols per liter, and

(4) at least one organic divalent sulfur compound selected from the group consisting of thio-diglycolic acid,  $\beta$ -thio-dipropionic acid, 1,1'-thio-bis-(2,2,2-trichloro-ethanol), (methylene-dithio)-diacetic acid, 1-ethyl-thioethanol, 2,2'-thio-diethanol,  $\alpha$ -amino- $\gamma$ -(methyl-thio)-butyric acid, bis(N- $\gamma$ -oxypropyl)-thiodipropylene glycol-dicarboxylic acid amide, S-(2-carboxyphenyl)-thio-glycolic acid, S-(8-chloro-1-naphthyl)-thioglycolic acid, (p-chlorophenyl-thio)-acetic acid, (2-methyl-3-chlorophenyl-thio)-acetic acid, (pentachlorophenyl-thio)-acetic acid, (2-nitro-4-acetamidophenyl-thio) - acetic acid, 2-( $\alpha$ -hydroxyethyl-thio)-4-ethylbenzoic acid, 3-carboxymethyl-thio-2-anthraquinone carboxylic acid (di-Na-salt), acetylene-dithio-salicylic acid, 4,4'-dinitro-diphenylsulfide-6,6'-disulfonic acid, 2,2'-thio-di(5-amino-benzene sulfonic acid), 2-thiophene carboxylic acid, 3,4-diphenyl-thiophene-2,5-dicarboxylic acid, 3-hydroxy-thionaphthene-2-carboxylic acid, 2-hydroxy-thionaphthene, 2-hydroxy-3-dibenzothiophen-carboxylic acid, 2,3-thionaphthenedion, 2-(p-aminophenyl)-5-sulfo-6-benzothiazole carboxylic acid, 2-amino-5-(6'-methyl-2'-benzothioazolyl)-1,3 - benzene disulfonic

14

acid, 2-(m-aminophenyl)-7-hydroxynaphtho-(2,3-d)-thioazole-5-sulfonic acid in an amount of between 0.001 and 5 g. per liter.

6. Process according to claim 5, wherein said plating bath additionally contains a member selected from the group consisting of methanol, phenol, and dioxane as solubilizer.

7. Process according to claim 5 wherein said plating bath additionally contains a member selected from the group consisting of sodium acetate, sodium nitrate, and sodium tartrate in an amount of between 5 and 200 g. per liter of buffering agent.

8. Process according to claim 5 wherein said plating bath additionally contains in solution a lead salt in an amount of between 0.001 and 1 g. per liter.

#### References Cited by the Examiner

##### UNITED STATES PATENTS

|    |           |         |                     |        |
|----|-----------|---------|---------------------|--------|
| 20 | 2,528,902 | 11/1950 | Moy et al. -----    | 204-49 |
|    | 2,844,530 | 7/1958  | Wesely et al. ----- | 204-49 |
|    | 2,994,369 | 8/1961  | Carlin -----        | 106-1  |
|    | 3,062,666 | 11/1962 | McLeod -----        | 106-1  |
|    | 3,096,182 | 7/1963  | Berzins -----       | 106-1  |

##### FOREIGN PATENTS

|         |        |                |
|---------|--------|----------------|
| 836,480 | 6/1960 | Great Britain. |
| 626,999 | 9/1961 | Great Britain. |

30 MORRIS LIEBMAN, *Primary Examiner.*

JOSEPH REBOLD, ALEXANDER H. BRODMERKLE,  
*Examiners.*